

# UNITED STATES PATENT OFFICE

FREDERICK M. BECKET, OF NIAGARA FALLS, NEW YORK, ASSIGNOR TO ELECTRO METALLURGICAL COMPANY, OF NEW YORK, N. Y., A CORPORATION OF WEST VIRGINIA.

## METHOD OF DEPHOSPHORIZING FERROTUNGSTEN.

1,081,569.

Specification of Letters Patent.

Patented Dec. 16, 1913.

No Drawing.

Application filed April 24, 1913. Serial No. 763,258.

To all whom it may concern:

Be it known that I, FREDERICK M. BECKET, a subject of the King of Great Britain, residing at Niagara Falls, in the county of 5 Niagara and State of New York, have invented certain new and useful Improvements in Methods of Dephosphorizing Ferrotungsten, of which the following is a specification.

10 This invention relates to methods of dephosphorizing ferrotungsten, particularly ferrotungsten which by reason of its high tungsten-content cannot economically be brought to the thinly-fluid condition required 15 site for continuous tapping or pouring.

As is well known, commercial ferrotungsten containing 75-80 per cent. or upward of tungsten is difficultly fusible, and requires the application of extremely high 20 temperatures in order to bring it to a fluid condition or to melt it into a homogeneous mass. The solidified alloy is however comparatively brittle, and can be easily ground or stamped into fragments or into grain or 25 powder form.

According to the present invention, the alloy, in suitably subdivided condition, is fed to a molten dephosphorizing bath, which is preferably but not necessarily maintained 30 by electrically-applied heat at a temperature sufficiently high to fuse or agglomerate the particles of the alloy, whereby the depolarized metal is obtained in compact form. The bath should be basic in character 35 in order to effect satisfactory dephosphorization, and should be of such composition as to avoid, so far as possible, transfer of the refractory metal from the alloy to the bath. It is therefore desirable that the bath 40 should consist of an ore of the refractory metal which enters into the constitution of the alloy, with such basic addition, usually lime, as may be required.

An illustrative example of my method is 45 as follows: Ferrotungsten, containing 75-80 per cent. of tungsten, is crushed to pass a 10-12 mesh screen, and is fed in a continuous stream to the surface of a molten bath consisting of scheelite and lime in approximately equal proportions. This bath is maintained by the passage therethrough of an electric current at such temperature as will suffice to fuse or at least to agglomerate

the purified alloy. The bath may be used until it becomes sluggish in its refining action, after which it is replaced by a fresh bath. During the operation the phosphorus-content of the bath gradually increases, and when a given bath has been used as long as is advisable under the particular circumstances, it is tapped from the furnace, permitted to cool, and treated as a high-phosphorus ore of tungsten; that is to say, it may be smelted with silicon or with carbon for preparation of a ferroalloy, 55 which, being comparatively high in phosphorus, may be purified by any desired method, for example as above described, or by any of the methods described in my co-pending application Ser. No. 728,498, filed 70 October 29, 1912. It will of course be understood that the reduction of phosphorus in smelting the phosphorized bath is by no means quantitative, so that it is often practicable to purify the ferroalloy obtained 75 by smelting the rejected baths by dephosphorization in fresh baths without involving any serious accumulation of phosphorus in the process. This is particularly the case when the ore employed for the fresh bath is 80 substantially free from phosphorus.

This method is chiefly applicable to the treatment of ferrotungsten which is low in carbon, inasmuch as a similar treatment of high-carbon ferrotungsten is apt to entail 85 a reduction of phosphorus from the bath, particularly when the bath is relatively high in phosphorus, with the result that the alloy is imperfectly dephosphorized. The applicability of the method is independent of 90 the tungsten-content of the alloy, and the method is directly applicable to the treatment of products having a tungsten-content of 94 to 98 per cent., such for example as the product known to the trade as "tungsten powder"; and the term "ferrotungsten" is herein used as including such products.

It is found that ferrotungsten, particularly when comparatively rich in tungsten, 100 cannot be satisfactorily dephosphorized by such methods as are applicable to the dephosphorization of steel, that is to say, by subjecting a body of molten ferrotungsten to the action of an overlying bath of basic 105 slag. According to the present method, the

ferrotungsten is brought in solid form into presence of the basic bath, and undergoes progressive heating in the bath, encountering during such heating the conditions which 5 accomplish the deposphorization.

I claim:-

1. The method of deposphorizing ferrotungsten, which consists in bringing the ferrotungsten in solid form into presence 10 of a molten basic oxidizing bath.
2. The method of deposphorizing ferrotungsten, which consists in bringing the ferrotungsten in solid form into presence of a molten basic oxidizing bath maintained 15 at a temperature approximating or above the fusing-point of the ferrotungsten.
3. The method of deposphorizing ferrotungsten, which consists in bringing the ferrotungsten in solid form into presence 20 of a molten basic oxidizing bath containing an oxygen compound of tungsten.
4. The method of deposphorizing ferrotungsten, which consists in bringing the ferrotungsten in solid form into presence of 25 a molten basic oxidizing bath containing an oxygen compound of tungsten, said bath maintained at a temperature approximating or above the fusing-point of the ferrotungsten.
30. 5. The method of deposphorizing fer-

rotungsten, which consists in feeding solid ferrotungsten in subdivided form to the surface of a molten basic oxidizing bath.

6. The method of deposphorizing ferrotungsten, which consists in feeding solid 35 ferrotungsten in subdivided form to the surface of a molten basic oxidizing bath maintained at a temperature approximating or above the fusing-point of the ferrotungsten.

7. The method of deposphorizing ferrotungsten, which consists in feeding solid ferrotungsten in subdivided form to the surface of a molten basic oxidizing bath containing an oxygen compound of tungsten. 40

8. The method of deposphorizing ferrotungsten, which consists in feeding solid ferrotungsten in subdivided form to the surface of a molten basic oxidizing bath containing an oxygen compound of tungsten, 50 said bath maintained at a temperature approximating or above the fusing-point of the ferrotungsten.

In testimony whereof I affix my signature in presence of two witnesses.

FREDERICK M. BECKET.

Witnesses:

C. P. TOWNSEND,  
E. DANIELS.

Correction in Letters Patent No. 1,081,569.

It is hereby certified that in Letters Patent No. 1,081,569, granted December 16, 1913, upon the application of Frederick M. Becket, of Niagara Falls, New York, for an improvement in "Methods of Deposphorizing Ferrotungsten," an error appears in the printed specification requiring correction as follows: Page 1, lines 32-33, for the word "depolarized" read *deposphorized*; and that the said Letters Patent should be read with this correction therein that the same may conform to the record of the case in the Patent Office.

Signed and sealed this 20th day of April, A. D., 1915.

[SEAL.]

J. T. NEWTON,

*Acting Commissioner of Patents.*